

Nov. 4, 1958

S. E. SEAMAN ET AL

2,859,210

## METHOD OF PRODUCING ALKALI CELLULOSE

Filed Dec. 10, 1956



2,859,210

**METHOD OF PRODUCING ALKALI CELLULOSE**Stewart E. Seaman, Osprey, Fla., and Stewart L. Seaman,  
White Plains, N. Y.

Application December 10, 1956, Serial No. 627,388

4 Claims. (Cl. 260—233)

This invention relates to a method of producing alkali cellulose to be used in the viscose process.

Pulp for making alkali cellulose is customarily obtained by the rayon or other viscose plants from pulp mills in the form or quality known as dissolving pulp. Such pulp has a high alpha cellulose content which is obtained in the pulp mill, in the usual sulphite process, for example, by drastic cooking and by caustic alkali treatments at elevated temperatures but at the expense of considerable loss of yield. The pulp is washed with water after each alkali treatment without any provision for recovery of the alkali. Following the cooking in the digester the washed unbleached pulp is customarily chlorinated for the purpose of substantially removing the lignin that has not been removed in the cooking operation, after which it is washed and in addition to the caustic treatments it is subjected to one or more sodium hypochlorite treatments for bleaching, followed in each instance by washing and finally it is customarily given a sulphur dioxide treatment and is washed, after which it is sheeted and dried, cut to size and baled. The loss in yield in such process for the production of dissolving pulp may be as high as 30%, and another economic factor of considerable importance is the loss of alkali used in the treatments.

The alkali content of alkali cellulose for proper xanthation must be approximately 15% and it is the practice in the rayon plant to steep the dissolving pulp in sheets of precise dimensions as obtained from the pulp mill in a caustic solution having a concentration of approximately 18%, thereby converting the pulp into alkali cellulose.

For the production of paper pulp in which the presence of a certain amount of hemi-cellulose is desirable, a less drastic cooking is employed followed by chlorination, a relatively mild caustic treatment and bleaching, the pulp being washed after each step.

It is the object of the present invention to produce from a low cost pulp a uniform, high alpha alkali cellulose at less cost than is entailed in present processes, with a high yield, high activity in subsequent viscose treatment and a high degree of polymerization (D. P.), and which produces a viscose containing, before filtration, very few imperfectly dissolved particles, usually termed "gels," "fiber gels," etc. and hence gives but little trouble in filtration and in the spinning operation.

The present invention contemplates that the caustic treatment of the pulp to solubilize the hemi-celluloses, that is, the beta and gamma cellulose content, pentosan type of products, etc., be performed under conditions which will effect the maximum production of alpha cellulose without subsequent reduction of the soda concentration and consequent precipitation of the hemi-celluloses.

In accordance with the invention the treatment to add the soda to convert the cellulose into alkali cellulose also serves to wash the high alpha cellulose and remove the dissolved hemi-celluloses and thus precipitation of

the hemi-celluloses is avoided. There is no loss of alkali and the loss in yield is minimized.

In brief, the invention contemplates the use of any sulphite or prehydrolyzed kraft chlorinated pulp substantially free of lignin and treating it with cold caustic, that is, caustic soda at substantially room temperature, the concentration of which is such as to produce maximum swelling of the fibers under which condition they are subject to maximum reaction with caustic soda to dissolve the hemi-celluloses. The refined cellulose is then pressed to the lowest practical press ratio and is washed with a stronger caustic soda which both removes additional dissolved hemi-celluloses remaining in the pulp after pressing and adds the additional soda required for optimum press xanthation. Finally it is pressed again to the optimum press ratio for satisfactory shredding for xanthation. In practice for both caustic treatments the pulp is converted into a slurry of fibers in the caustic, and delivered into a tank where it is held at a temperature between 20° C. and 50° C. in a proper state of agitation for the required time.

It is contemplated for this purpose to use pulp that has been produced by either the sulphite or prehydrolyzed kraft process and which has been chlorinated for the purpose of substantially removing the lignin which has not been removed in the cooking operation to yield a cellulose of high activity and high D. P. In other words the pulping process to this stage may be in accordance with the treatment for the production of paper pulp.

If the viscose produced from the cellulose is to be used for tire cord, for example, no bleaching is necessary and the chlorination may be followed by a mild alkali treatment under somewhat elevated temperature to remove the lignochlorine and other dark color ingredients which were dissolved by the chlorination and are not completely soluble in acid or water condition. Where bleaching for whiteness is desirable it may follow the chlorine treatment.

The pulp is then pressed and sheeted without any requirement as to sheet size or moisture content, except that the moisture content must be exactly known, and is delivered to the viscose plant where it receives the refining and alkalizing treatments above mentioned.

The unbleached pulp should preferably be cooked to a low chlorine number, experience having shown that 2½% to 3% chlorine number yields an unbleached pulp sufficiently purified, with optimum activity and a sufficiently high degree of polymerization.

In this way a much lower cost pulp is supplied by the pulp industry for viscose use than has heretofore been the case. It has been customary in producing dissolving pulp for viscose use to spend considerable effort toward making a very uniform sheet of uniform thickness, dried to a carefully controlled low and uniform moisture content and carefully cut to uniform sheet size. Low moisture content, less than 10% tends to reduce the reactivity of cellulose.

In accordance with the present invention the chlorinated pulp, either unbleached or bleached to any desired degree, need not be put into any precise condition for shipping, with any particular attention to sheet formation, sheet thickness, specific moisture content or specific sheet size. In these respects the usual practice for supplying paper pulp may be followed. As a matter of convenience it will be sheeted but it need be dried only to that point providing optimum economy for shipping. A moisture content of from 10 to 20 percent has been found practicable.

It is known that, for any given temperature, maximum swelling of cellulose occurs at about 9½% caustic soda. At this maximum point of swelling the individual fibers

are subject to optimum reaction with caustic soda for removal of hemi-celluloses. Since ordinarily, as above mentioned, the pulp prepared at the pulp mill will contain on an average approximately 15% of moisture, it has been found practical to use a concentration of caustic soda for the first treatment of around 10%, thus providing an effective concentration of substantially 9.8% which for all practical purposes produces the maximum swelling.

In our preferred process we add pulp having a known amount of cellulose and containing about 15% of water to a 10% caustic soda solution which provides an effective concentration of about 9.8% at a properly calculated consistency. A 6% slurry is formed in a "Hydrapulper" or similar device which disperses each individual fiber into the caustic whereby optimum treatment is obtained.

The slurry is dropped into an agitating tank along with enough 10% caustic to bring the slurry to a consistency of around 1.5%.

The 1.5% slurry is formed into a web and passed through a suitable press, for example, that described in copending application Serial No. 566,844 by which it is reduced to a very low press ratio of between 2 and 3½ to 1, preferably around 2 or 2.5 to 1, in order to express the maximum amount of hemi-celluloses.

The pressed alkaline pulp is then delivered to a second agitating tank along with a sufficient volume of approximately 16% caustic, specifically 15.3%, to provide a slurry of about 1.5% consistency.

The slurry also is formed into a web and passed through a suitable press, for example, that described in said copending application, by which it is reduced to that press ratio suitable for shredding prior to xanthation, for example, from 2½:1 to 3½:1.

The second caustic treatment using about 16% caustic removes more hemi-cellulose from the highly swollen fibers, thus yielding a product with a higher alpha cellulose content and providing an alkali cellulose containing around 15% NaOH which is best for xanthating.

### EXAMPLE I

*Effect on alpha cellulose content by steeping with 11% concentration NaOH at 20° C. and 40° C.*

|                           | 11% Na OH,<br>20° C. | 11% Na OH,<br>40° C. |
|---------------------------|----------------------|----------------------|
| Alpha Cellulose:          |                      |                      |
| Unbleached.....percent    | 87.2                 | 87.2                 |
| After Chlorination.....do | 86.1                 | 86.1                 |
| After Alkali.....do       | 98.1                 | 97.2                 |
| Degree of Polymerization: |                      |                      |
| Unbleached.....           | 1,600-1,700          | 1,600-1,700          |
| After Alkali.....         | 1,465-1,500          | 1,550                |
| Pentosans:                |                      |                      |
| Unbleached.....percent    | 4.58                 | 4.58                 |
| After Alkali.....         | 1.29                 | 0.94                 |

No gels in viscose—untreated fibers negligible.

### EXAMPLE II

*Effect on alpha cellulose content by steeping with 11% concentration NaOH at 20° C. with another make of pulp with three different tests for check results*

|                         | 11%<br>NaOH,<br>20° C. | 11%<br>NaOH,<br>20° C. | 11%<br>NaOH,<br>20° C. |
|-------------------------|------------------------|------------------------|------------------------|
|                         | Percent                | Percent                | Percent                |
| Alpha Cellulose:        |                        |                        |                        |
| Unbleached.....         | 86.6                   | 86.6                   | 86.6                   |
| After Chlorination..... | 88.55                  | 88.55                  | 85.55                  |
| After Alkali.....       | 98.02                  | 99.12                  | 98.88                  |

### EXAMPLE III

*Effect on alpha cellulose content by steeping in several steps with 18% concentration NaOH at 20° C.*

|                           | Alpha cellulose, percent |
|---------------------------|--------------------------|
| Unbleached pulp.....      | 86.6                     |
| After chlorination.....   | 85.55                    |
| After first steep.....    | 94.8                     |
| After second steep.....   | 98.0                     |
| 10 After third steep..... | 98.8                     |

### EXAMPLE IV

*Effect on alpha cellulose content by steeping with 10% concentration NaOH at 20° C. followed by a second steeping with 16% concentration NaOH at 20° C.*

|                          | Alpha cellulose, percent |
|--------------------------|--------------------------|
| Unbleached.....          | 86.6                     |
| After chlorination.....  | 85.5                     |
| After alkali 10%.....    | 98.7                     |
| 20 After alkali 16%..... | 99.2                     |

Example IV shows the percentage of alpha cellulose obtained by a treatment with a high swelling concentration of caustic followed by a treatment with a concentration which will provide an alkali cellulose having the required percentage of NaOH.

The best dissolving pulp produced by pulp mills using conventional methods has an alpha cellulose content of 96% or thereabouts and has suffered a loss of from 20 to 33% in passing from chlorinated pulp to the finished product. As compared with this the cellulose at the end of the 9.8% slurry steeping is refined to an alpha cellulose content of 98% or more and at the end of the 16% caustic treatment to about 99% alpha cellulose with a loss not exceeding 19% from the original chlorinated pulp.

The accompanying drawing illustrates diagrammatically an apparatus for the continuous production of alkali cellulose in accordance with the method of the invention. A weighed amount of chlorinated pulp substantially free of lignin is introduced into a pulper 1 of a conventional type, such as a "Hydrapulper," into which has previously been introduced from a supply tank 2 a determined amount of 10% NaOH. A slurry of the proper consistency results from the vigorous agitation in pulper 1, whereupon the slurry is reduced in consistency by additional NaOH from supply tank 2 to an optimum consistency for forming a uniform web for pressing and is discharged into steeping tank 3 in which the treatment is continued with effective stirring.

From the tank 3 the slurry is pumped to a web former 4 and is delivered in the form of a continuous web into the nip of press rolls 5 and pressed to a low press ratio. The liquor expressed from the web by press rolls 5 is delivered by line 6 to dialyzers 7.

From the first press 5 the web is delivered by conveyor 8 into a second steeping tank 9 having a suitable agitator and into which NaOH at a concentration of 16% is fed by line 10 as needed to maintain the proper consistency. The treatment in tank 9 is continued for substantially the same time as in tank 3. From tank 9 the alkali cellulose slurry is pumped to web former 11 and is delivered in the form of a continuous web into the nip of press rolls 12 in which it is again pressed to a low press ratio and from which it passes on to a conveyor 13 for delivery to the shredder.

The press liquor from press 12 is delivered by line 14 to supply tank 2. In order to obtain a concentration of 10% in the supply tank, sufficient recovered caustic at a concentration of about 5% is delivered from the dialyzers by line 15 into the supply tank 2.

In this way a continuous counter-current cyclic process is performed.

From the first press 5 the expressed caustic soda containing the maximum amount of hemi-cellulose is pumped

to dialyzers where the 10% concentration is reduced to about 5%, the hemi-cellulose is removed and the dilute 5% caustic soda is pumped to supply tank 2.

Dependent upon the alpha cellulose content of the chlorinated pulp entering the process, the percentage of hemi-cellulose dissolved during treatment will reach a balance of approximately 3% in the first caustic soda treating tank. Additional hemi-cellulose as produced will be removed by dialyzers from the pressed caustic resulting in the hemi-cellulose balance indicated. The second caustic soda treatment of the highly purified cellulose produces alkali cellulose and at the same time results in further solution of hemi-cellulose. Because of the high alpha cellulose content of the pulp in the steeping tank a hemi-cellulose balance of about 0.2% is attained. This very low hemi-cellulose content in the steeping caustic results in an alkali cellulose containing a very minimum of hemi-cellulose after pressing to contaminate the regenerated cellulose finished products. Minimum hemi-cellulose content is required to yield maximum strength and fatigue value of the yarn.

What is claimed is:

1. The method of producing alkali cellulose having a high degree of polymerization for use in the viscose process comprising first forming a slurry of a chlorinated pulp of high degree of polymerization and substantially free of lignin with a sodium hydroxide solution having an effective alkali concentration of substantially 9½% and maintaining the slurry for substantially 15 minutes at a temperature between 20° and 50° C. and producing a maximum swelling of the fiber, pressing the pulp so treated

to a press ratio of between 2 and 3.5 to 1, then forming a slurry of the pressed pulp with a second sodium hydroxide solution of higher concentration and maintaining the slurry for substantially 15 minutes at a temperature between 20 and 50° C. and pressing the product of the second causticizing to a press ratio of between 2 and 3.5 to 1, the concentration of said second caustic solution being sufficient to produce an alkali cellulose having an alkali content of not substantially less than 15% after pressing.

2. The method defined in claim 1 in which the concentration of the caustic solution of the first treatment is not substantially less than 9½% nor more than 11% and the treatment is continued for a period of substantially 15 minutes at not less than 20° C. nor more than 50° C.

3. The method defined in claim 2 in which the concentration of the caustic solution of the second treatment is substantially 16% and the second treatment is continued for substantially 15 minutes at not less than 20° C. nor more than 50° C.

4. The method defined in claim 3 in which the caustic solution in both slurry treatments is free of extraneous oxidizing agent, thereby retaining a high degree of polymerization.

References Cited in the file of this patent

UNITED STATES PATENTS

|    |           |               |               |
|----|-----------|---------------|---------------|
| 30 | 1,814,543 | Blanco et al. | July 14, 1931 |
|    | 1,955,092 | Richter       | Apr. 17, 1934 |
|    | 2,392,269 | Schmitz       | Jan. 1, 1946  |